

## UNITED STATES PATENT OFFICE

2,042,971

METHOD OF MAKING ELECTRICAL RESIST-  
ANCE ELEMENTS AND ALLOYS THERE-  
FORJames L. Thomas, Garrett Park, Md., assignor to  
the Government of the United States, repre-  
sented by the Secretary of CommerceNo Drawing. Application November 22, 1934,  
Serial No. 754,310

1 Claim. (Cl. 201—76)

(Granted under the act of March 3, 1883, as  
amended April 30, 1928; 370 O. G. 757.)

The invention described herein may be manufactured and used by or for the Government of the United States for governmental purposes only without the payment of any royalty thereon.

5 This invention relates to a new and improved electrical resistance element and method of making the same, as well as the preparation of the alloy therefor.

Generally, in electrical measuring apparatus, 10 coils of wire are utilized and difficulty has always been encountered in obtaining a wire whose resistance remains stable or substantially constant. It is known that resistance changes with age and also with ordinary changes in laboratory 15 temperature. The change which takes place with age may be due to chemical action of the air upon the surface of the wire, or to changes in the crystal arrangement therein.

Further, besides the stability, resistance alloys 20 should have low temperature coefficients of resistance in order that they may be readily measured to a high precision.

To the best of my knowledge, no alloy has been developed which is entirely free from changes in 25 resistance with time or with temperature, but special alloys have been developed for which the changes in resistance with temperature and time are comparatively small. "Manganin", an alloy of copper, manganese and nickel is the 30 alloy most generally used for this purpose at present, but this alloy does not possess the desired qualities to a sufficiently high degree.

I have conducted experiments with an alloy 35 consisting mostly of gold with a small addition of chromium. Specifically, my research and tests have included a number of different alloys composed of gold with the addition of approximately from 1.5 to 5 percent of chromium by weight. As a result of the tests I have found the most desirable mixture is approximately 2.1 percent of 40 chromium and the remainder gold. Moreover, I have discovered that the addition of 1.5 to 5 percent of chromium to gold produces alloys having very small temperature coefficients of electrical resistance and that the temperature coefficient of the alloys depends upon the proportions of the two ingredients and the method of forming the finished article.

The first difficulty encountered was to 45 discover a method by which the two ingredients

could be properly alloyed, and after a number of tests, I found the best method is to melt the gold and chromium together, in graphite crucibles, under a heavy coating of borax, the coating of borax being for the purpose of excluding air and thus preventing oxidation of the alloy. The crucibles are preferably heated by means of an induction furnace, and when a temperature of about 1200° C. is reached, the alloys are poured into the graphite molds, the 10 graphite crucibles and molds being preferable because graphite absorbs oxygen and will assist in the prevention of oxidation. While other methods of preparation would serve the purpose, such as alloying the metals in a vacuum or in an atmosphere of dry hydrogen, I prefer to use the one just described because of its simplicity and the good results obtained. The use of a vacuum or dry hydrogen atmosphere requires a complicated and expensive apparatus and does not render any 15 better, if as good, results as my preferred method.

After being molded, the ingots may be first hot-forged into the form of rods 5 or 6 mm. square. Then they are preferably cold-rolled and swaged to a diameter of 0.75 mm., after which they are 25 drawn down to the required size through appropriate dies, such as sapphire dies. During the rolling and swaging the material may be annealed four or five times, but in my preferred method the wire is not annealed during the process of 30 drawing.

After the wire has been formed into a coil it is put through a baking process which has the effect of aging it artificially—that is to say, when I used the 2.1 percent chromium coils they were 35 baked for several hours at a temperature of approximately 200° C., and after this baking the change in resistance, with time, is much slower than for unbaked coils.

This baking has another effect besides that of 40 artificially aging the resistance of the coil. When the coils are baked at a temperature of from 100° C. to 500° C. the temperature coefficients of resistance are decreased. The amount of this decrease in temperature coefficient was found to 45 depend on both the baking temperature and length of time the coils are baked. By properly choosing the temperature and time of baking it is possible to adjust the temperature coefficient to zero for coils having a positive temperature co- 50

efficient before baking. For example, an unbaked coil of the 2.1 percent chromium alloy had a temperature coefficient of 80 parts per million per degree C. Its temperature coefficient of resistance was reduced to zero by baking at 200° C. for about 5 hours.

The following table is illustrative of the temperature-resistance changes of a 10-ohm coil of the 2.1 percent chromium alloy baked at a temperature of 200° C. to bring its value to zero:

|    | Temperature | Resistance           |
|----|-------------|----------------------|
| 15 | 20° C.      | 9.99561 <sub>1</sub> |
|    | 22.5        | 9.99561 <sub>2</sub> |
|    | 25          | 9.99561 <sub>1</sub> |
|    | 27.5        | 9.99561 <sub>0</sub> |
|    | 30          | 9.99561 <sub>1</sub> |

The resistance of this coil was substantially independent of temperature throughout the entire interval 20-30° C. With manganin a minimum variation of about 10 parts per million would have been expected in this temperature interval, which is nearly a hundred times that of the 2.1 percent chromium alloy. In testing 10-ohm and 100-ohm coils the temperature-resistance curves were found to be substantially identical in each case.

The baking of the alloyed element is the essen-

tial step in its artificial aging and has the advantage of doing away with, or at least substantially reducing, the aging that would ordinarily take place as the element ages with time.

When manganin is used, in the construction of resistance standards, the coils are usually kept for a year or more in order to reach a reasonably stable state, but with my alloy and the herein-described process of making the coils, this aging is not necessary, and, obviously, is greatly preferable to the manganin.

As will be evident to those skilled in the art, my invention permits of various modifications of the method employed and of changes in percentage of elements in the alloy without departing from the spirit thereof or the scope of the appended claim.

What I claim is—

The method of making an electrical resistance element which includes the steps of combining 20 gold and chromium, the chromium being in the percentage of from 1 to 5 percent and the remainder being gold, forming the wire into wire strands and adjusting the temperature coefficient of said resistance element to zero by baking said 25 element in an atmosphere of air at a temperature of from 100° C. to 500° C.

JAMES L. THOMAS.